

1

2,994,661

## PREPARATION OF DIESTER OIL SOLUTIONS OF MINERAL OIL-FREE BASIC ALKALINE EARTH METAL MAHOGANY SULFONATES

Lee V. Brown, Chicago, Ill., assignor to Sinclair Refining Company, New York, N.Y., a corporation of Maine  
No Drawing. Filed Apr. 9, 1958, Ser. No. 727,250  
4 Claims. (Cl. 252—33)

This invention relates to a process for the manufacture of an additive solution. More particularly, my invention pertains to a process for the manufacture of an additive concentrate in a diester synthetic lubricant vehicle.

Previous work with diester base synthetic lubricants has shown that mineral lubricating oil can be incompatible with diesters of lubricating viscosity. Thus the use of conventional mineral lubricating oil diluted additives in the diester base liquids requires that the additives be deoiled. Investigations with diester base lubricants using deoiled conventional additives established that the method of compounding is an element of prime importance particularly when incorporating additives which have constituents reactive with the diester lubricant base. For instance, additives frequently employed in the diester lubricants are base oil-soluble, basic mahogany sulfonates of the alkaline earth metals especially those of calcium and barium. In designating these sulfonates as basic I refer to the fact that the alkaline earth metal is present in an amount in excess of that theoretically required to react with the sulfonic acid from which it was made, for instance, at least about 1.2 equivalents. In the case of the barium sulfonates there is usually at least about 1.5 equivalents of barium in the sulfonate and usually the basic sulfonates do not have more than about 5 equivalents of alkaline earth metal.

Mineral oil-free basic alkaline earth metal mahogany sulfonates can be dissolved directly in a diester vehicle only after prolonged agitation and heating. The use of a volatile solvent such as benzene to first dissolve the sulfonate followed by mixing with the diester and topping to remove the benzene solvent, results in saponification of the diester and subsequent gelation of the mixture.

The purpose of this invention is to overcome these difficulties by providing a method for incorporating mineral lubricating oil-free, basic alkaline earth metal mahogany sulfonates into diester synthetic lubricants. Further this invention provides a method of producing a concentrate of a mineral oil-free, basic alkaline earth metal mahogany sulfonate in a diester synthetic lubricant vehicle where the sulfonate is, for example, about 25 to 75% of the composition. This concentrate is compatible with synthetic diesters of lubricating viscosity and the sulfonate does not deleteriously react with the diester of the concentrate or a diester lubricant base oil to which it is added. These concentrates are clear, stable and easily pumpable to facilitate handling, storage and blending into synthetic lubricants of the diester type.

This invention consists essentially of dissolving in a volatile liquid hydrocarbon solvent a mineral oil-free mahogany sulfonate, for instance formed by the process of reacting an oil-soluble sulfonic acid petroleum oil with ammonia, an alkali metal such as sodium, lithium or potassium, or an alkaline earth metal such as calcium or barium; and extracting the resulting sulfonate as with alcohol, say of 1 to 3 carbon atoms, and water. The ammonium and alkaline metal sulfonates are soluble in a 50 volume percent solution of isopropanol in water. The liquid hydrocarbon solvent is compatible with diester oils of lubricating viscosity and boils primarily below about 350° F., preferably below about 300° F. The solvent usually contains a large proportion of aromatic con-

2

stituents. The resulting solution is reacted with an excess of a basic inorganic compound of an alkaline earth metal such as the oxides, hydroxides and carbonates, to produce the corresponding mineral lubricating oil-free, basic alkaline earth metal mahogany sulfonate such as that of barium. The oil-free basic alkaline earth metal mahogany sulfonate is carbonated by contact with carbon dioxide while obtaining a pH of not more than about 8.5 by carbonation. The diester synthetic lubricant vehicle, formed from alcohols and polycarboxylic acids, is then added. The resulting product is distilled to remove the solvent and recover the additive concentrate.

In my process the oil-free mahogany sulfonate (which can be derived from conventional oleum or sulfur trioxide treatment of mineral oil distillates) is dissolved in a volatile hydrocarbon solvent such as toluene, aromatic naphtha or heptane with generally a solvent to sulfonate ratio range of about 1:1 to 5:1 or more. The preferred solvent to sulfonate range in my invention is about 1.25 to 3.0:1. The resulting solution is reacted with an excess of a basic inorganic compound of an alkaline earth metal to produce the corresponding basic alkaline earth metal mahogany sulfonate. The mineral lubricating oil-free alkaline earth metal mahogany sulfonate is then carbonated, for instance in a temperature range of about 70° F. to 220° F. The preferred temperature range of carbonation is about 100° F. to 150° F. The preferred pressure range for the absorption of carbon dioxide which is aided by higher pressures would be from about atmospheric pressure to about 10 atmospheres pressure. During carbonation a pressure range from about atmospheric pressure to about 70 atmospheres can successfully be employed. The solution is carbonated to give a maximum pH of about 8.5. The preferred pH range for my invention is about 7.5 to 8.5. The diester vehicle is then added to my carbonated solution. The diester vehicle of lubricating viscosity is formed from alcohols and polycarboxylic acids. Among the dicarboxylic acids employed are those having from 2 to 12 carbon atoms such as adipic, azelaic, suberic, alkenyl succinic and sebacic acids. The alcohols employed usually contain 4 to 20 carbon atoms such as butyl, hexyl and 2-ethylhexyl and dodecyl alcohols; preferably the alcohol contains 6 to 12 carbon atoms. The resulting solvent can be distilled by the conventional methods of either batch or continuous distillation. Topping can be accomplished at reduced pressures to remove the last trace of volatile solvent. During distillation the solution should not exceed a maximum temperature of about 350° F., preferably not above about 300° F.

The following example will serve to illustrate my invention but it is not to be considered limiting.

*Example.*—777 pounds of sulfonic acid oil is produced by the treatment of a 150 lb. oleum/bbl. of dewaxed Mid-Continent 250 SSU/100° F. lubricating oil distillate. The acid oil is charged in an agitator and neutralized with 14.1 lbs. of ammonium hydroxide, 56.4 lbs. of water and 67.3 lbs. of 99 percent isopropyl alcohol are added to the agitator at 140° F. and then two hours' settling time is allowed. The lower alcohol layer is withdrawn. Then 6,000 grams of the alcohol extract is diluted with 50 percent isopropyl alcohol-water solution to a total volume of 8 gallons. The alcohol solution is extracted six times with 4,000 cc. charges of hexane which are discarded and the remaining isopropyl alcohol is topped off at about 208° F. The sulfonate-water residue from the alcohol recovery step is mixed with about 2 gallons of toluene and neutralized with 1,080 grams of barium oxide (300 percent of theoretical). The remaining water is topped off and the toluene solution is filtered. The solution is then distilled and the toluene removed with a resulting recovery of about 5 lbs. of mineral oil-free

solid basic barium sulfonate. Analysis of the basic barium sulfonate discloses:

Percent barium ..... 22.2  
Base No. to pH -4 ..... 78.1

Next 1513 grams of oil-free barium sulfonate is dissolved in 2323 grams of toluene and carbonated at atmospheric pressure with carbon dioxide gas at about 100° F. until a pH of 8.4 is obtained. Then 1513 grams of di-2-ethylhexyl sebacate (Plexol 201) is added to the toluene solution and the toluene is distilled off at atmospheric pressure and the material is topped at 300° F. and 10 mm. Hg. The product is a clear dark liquid without evidence of insolubles such as gels.

The following example will serve to illustrate a conventional process for manufacture of an additive concentrate in a synthetic diester lubricant vehicle.

*Example.*—20,024 grams of oil-free ammonium mahogany sulfonate are mixed with 8 gallons of toluene and 1 gallon of water. The resulting solution is contacted with 2450 grams of barium oxide (300 percent of theoretical), and then dehydrated and filtered. Sufficient of the toluene solution is then added to 3632 grams of di-2-ethylhexyl sebacate to give a composition containing 3632 grams of the oil-free basic barium sulfonate. The temperature is then raised to facilitate the topping off of toluene. As the solution reaches a temperature of about 240° F., well below required temperature for toluene topping, an insoluble gel is formed. This gel is essentially a barium salt of sebacic acid and free alcohol.

The product of my invention is a clear dark liquid which has no evidence of gelation and is essentially void of insolubles while the commercial process example exhibited high viscosity and saponification of the diester and then subsequent gelation of the mixture.

I claim:

1. A method of producing a solution of mineral oil-free basic alkaline earth metal mahogany sulfonate in a

diester lubricant vehicle which consists essentially of reacting a mineral lubricating oil-free mahogany sulfonate dissolved in a volatile hydrocarbon solvent boiling below about 350° F., with a basic inorganic alkaline earth metal compound to produce a basic alkaline earth metal mahogany sulfonate solution, carbonating the solution to a pH of not more than about 8.5, adding to the carbonated solution a diester vehicle of lubricating viscosity formed from alcohol having 4 to 20 carbon atoms and dicarboxylic acid of 2 to 12 carbon atoms, and distilling the resulting solution to remove the solvent.

2. The method of claim 1 in which the alkaline earth metal is barium.

3. The method of claim 1 in which the diester lubricant vehicle is di-2-ethylhexyl sebacate.

4. A method of producing a solution of mineral oil-free basic barium mahogany sulfonate in a diester lubricant vehicle which consists essentially of reacting a mineral lubricating oil-free ammonium mahogany sulfonate dissolved in toluene, with an oxide of barium to produce a basic barium mahogany sulfonate solution, carbonating the solution to a pH of not more than about 8.5, adding di-2-ethylhexyl sebacate to the carbonated solution, and distilling the resulting solution to remove the solvent.

#### References Cited in the file of this patent

##### UNITED STATES PATENTS

30 2,723,236 Asseff et al. ..... Nov. 8, 1955  
2,861,951 Carlyle ..... Nov. 25, 1958

##### FOREIGN PATENTS

786,167 Great Britain ..... Nov. 13, 1957  
787,459 Great Britain ..... Dec. 11, 1957

##### OTHER REFERENCES

"I. and E. Chem.," vol. 46, No. 5, May 1954, pages 1035-1042.